

June 8, 1943.

R. J. PIERSOL

2,321,238

SMOKELESS BRIQUET

Filed Aug. 30, 1941



FIG. 1.



FIG. 2.



FIG. 3.

INVENTOR  
Robert J. Piersol

## UNITED STATES PATENT OFFICE

2,321,238

## SMOKELESS BRIQUETTE

Robert James Piersol, Champaign, Ill.

Application August 30, 1941, Serial No. 408,957

3 Claims. (Cl. 44—10)

An object of my invention is to provide a smokeless briquette from bituminous coal without carbonization.

More particularly it is the object of the invention to provide a smokeless briquette from bituminous coal fines rich in fusain, which is a banded ingredient in bituminous coal. Fusain is commonly known as coal charcoal or natural charcoal. Fusain is supposed to have originated from wood charcoal produced by prehistoric forest fires at the geologic period during which the coal beds started to form. Fusain is a smutty black powder which largely forms the parting planes in banded bituminous coals. Fusain is very high in fixed carbon and very low in volatile matter.

A further object of the invention is to provide a smokeless briquette from products such as deduster dust and sludge, which are discarded in the cleaning of bituminous coal. Such products are rich in fusain due to the pulverant and friable nature of fusain, which tends to concentrate in the very fine sizes of bituminous coal.

A further object of my invention is the conservation of natural resources by the processing of a smokeless briquette from a waste product produced in the cleaning of coal, such waste product being discarded because it has no market in its raw state and the quantity of such waste product being of very large tonnages, with annual production in excess of one million tons for the State of Illinois.

A further object of the invention is to provide a smokeless fuel by briquetting bituminous coal fines, rich in fusain, without the use of a binder by the process disclosed in my Letters Patent No. 2,021,020, using a briquetting press disclosed in my Letters Patent No. 2,119,243, thus eliminating the smoke produced from the usual asphalt binder.

A further object of my invention is to provide a smokeless fuel by briquetting coal fines, rich in fusain, with the use of a smokeless binder, such as starch.

More particularly it is my object to provide a smokeless briquette from bituminous coal fines, rich in fusain, by the use of a briquetting process which does not add a smoke producing ingredient to the briquette.

With these and other objects in view my invention consists of both a smokeless briquette and the process for making a smokeless briquette from bituminous coal fines, rich in fusain, whereby the objects contemplated are obtained, as herein-after more fully set forth, pointed out in my

claims, and the effect of various percentages of fusain on the smoke producing characteristics of the resultant briquette is illustrated in the accompanying drawing, in which:

Figure 1 is a graph which shows the normal concentration of fusain in the very fine sizes of coal. This particular graph is for deduster dust from a typical dry coal cleaning plant located in southern Illinois. The deduster dust is a waste product which consists of the very fine sizes of coal, which are air separated from stoker coal.

Figure 2 is a graph which shows the influence of the percentages of fusain in the various screen sizes of deduster dust on the smoke index, which is a quantitative measure of the smoke producing potentiality of the resultant briquette made without an added binder.

Figure 3 is a graph which likewise shows the influence of the percentage of fusain on the smoke index of the resultant briquettes, the hand picked pure fusain being blended in various percentages with fusain free high volatile coal.

Analysis of the above illustrated experimental data shows that the percentage of fusain increases from about 4 per cent, which is approximately the average percentage of fusain in the corresponding lump coal, up to 37.5 per cent for the very finest sizes of deduster dust and that the smoke index of the resultant briquette diminishes linearly with the increased percentage of fusain, vanishing at 40 per cent fusain.

In general it is found that the smoke index of natural coals, and briquettes made from natural coals, decreases linearly with decrease of percentage of volatile matter and therefore the percentage of volatile matter has become the criterion for acceptance of smokeless coal under certain smoke abatement ordinances, one value being 23 per cent or less, volatile matter; the resultant smoke from coal of said volatile matter corresponding to a smoke index of 2300. Therefore the term smokeless is used herein to designate such a coal fuel.

One skilled in the art of processing smokeless products from coal would therefore expect that the addition of fusain to high volatile coal would decrease the smoke index of the resultant briquette only to the extent that the percentage of volatile matter would be lowered on account of the very low volatile content of fusain which is usually 5 per cent or less. However, experiment proves, as illustrated in Figure 3, that a briquette containing 15 per cent fusain possesses a smoke index of 2300 units, although chemical analysis

shows that this briquette contains over 30 per cent volatile matter.

After having established experimentally that the smoke produced from a briquette made from coal fines rich in fusain is several fold less than that which would be predicted from the resultant decrease of percentage of volatile matter due to the fusain, I have found that this unexpected decrease in smoke is due to a catalytic reaction of the fusain which reacts in combustion in a manner similar to activated charcoal, thereby accelerating the combustion of the low temperature fraction of the volatile matter which is the normal smoke producing ingredient of bituminous coal.

The process for making smokeless briquettes from coal rich in fusain consists of concentration of fusain in the very fine sizes of coal by means of dry dedusting or wet washing, and of the removal of oversize fines, usually over 20 mesh in size, in order that the material contain 15 per cent or more fusain, and of briquetting without added binder or of briquetting with a smokeless binder. If the product, rich in fusain, is briquetted without binder, the preferred method is to preheat the product to a temperature somewhat less than its initial softening point and to apply impact pressure of relatively high magnitude in order to flow the product into a briquette. I find that one preferred set of briquetting conditions consists of a temperature of about 350 degrees centigrade, a pressure of about 30,000 per square inch applied for a period of about one tenth of a second in the specially designed press described in my Letters Patent No. 2,119,243. If the product, rich in fusain, is briquetted with a smokeless binder, usual briquetting processes and usual briquetting equipment may be used.

My invention, herein described, is now being

commercialized on a large scale and the resultant smokeless briquette has been accepted officially by the city of St. Louis because large scale combustion tests show that the smoke produced by this briquette compares favorably with that produced by natural smokeless coals. It is not my intent to limit the scope of this invention to the particular methods herein described for making a smokeless briquette from coal fines rich in fusain nor to limit the percentage of fusain in the smokeless briquette to that herein described. On the other hand the method of making a smokeless briquette from coal fines rich in fusain and the smoke characteristics of the resultant briquette can be modified considerably without departing from the real spirit and purpose of my invention and it is the purpose and it is my intention to cover by my claims any modifications which may be reasonably included within the scope of my invention.

I claim as my invention:

1. A briquette which consists of from 60 to 85 per cent high volatile bituminous coal and of from 15 to 40 per cent fusain, and with a range of smoke content between 2300 and zero smoke index units.
2. A briquette composed of high volatile bituminous coal and admixed fusain with an optimum proportion of about 20 per cent fusain, and with a smoke content of about 1800 smoke index units.
3. A process for manufacture of briquettes, with smoke index less than 2300, from high volatile smoke producing bituminous coal, consisting of concentration of fusain to proportions of over 15 per cent by means of size classification to particle diameter of less than 0.007 inch and of briquetting without use of smoke producing binder.

ROBERT JAMES PIERSOL.